

Patented May 6, 1924.

1,492,712

# UNITED STATES PATENT OFFICE.

BETHUNE G. KLUGH, OF CHICAGO, ILLINOIS, ASSIGNOR TO FEDERAL PHOSPHORUS COMPANY, OF BIRMINGHAM, ALABAMA, A CORPORATION OF ALABAMA.

## PROCESS FOR THE PRODUCTION OF PHOSPHORUS AND POTASH COMPOUNDS.

No Drawing. Application filed September 20, 1920, Serial No. 411,483. Renewed August 23, 1922. Serial No. 583,939.

*To all whom it may concern:*

Be it known that I, BETHUNE G. KLUGH, a citizen of the United States of America, residing at Chicago, in the county of Cook and State of Illinois, have invented certain new and useful Improvements in Processes for the Production of Phosphorus and Potash Compounds, of which the following is a specification.

- 10 This invention relates to the electric smelting of a mixture of natural phosphate, potassium bearing silicate or aluminate rock and carbon to the end that the phosphorus and potash content of the charge will be simultaneously volatilized, the elemental phosphorus oxidized in the presence of the volatilized potash and the two constituents collected together as phosphoric acid and potash.
- 20 My invention further contemplates the utilization, in processes for the electric smelting of phosphatic materials with or without iron, of potash bearing shale or silicate or aluminate rock to furnish the required quantity of silica for the flux which has heretofore been supplied by sand or silicate rocks having no recoverable values.

My invention further contemplates the production of a compound of phosphorus and potash as a by-product of an electric furnace engaged in the production of commercial ferro-phosphorus, this being accomplished by the charging of a potash bearing silicate instead of sand and the control of the temperature and stock depth in the furnace upon the principles defined in my pending application, Serial No. 388,822, filed June 14th, 1920.

I am aware that it has been proposed to treat potassium bearing rocks, such as feldspar or muscovite, by heating them with natural phosphates, the principal constituent of which is tricalcium phosphate, preferably in an electric furnace and at temperatures up to 2000° C. to produce potassium phosphate. These processes do not contemplate the admixture of carbon or any other reducing agent with the charge and, as described, are conducted with no reduction of the phosphorus. Such processes are based upon the assumption that the phosphorus passes out as phosphorus oxides and the potassium as potassium oxides or other volatile compounds thereof. Furthermore,

these existing processes make no mention of any ratio of the silica and lime in the reacting mixture.

My process hereindescribed differentiates from such above described existing processes in that I have found that it is essential that the phosphorus must be reduced in order that it be volatilized in commercial proportions and that the ratio of the silica and lime in the charge must be accurately proportioned in order that the quantity of phosphorus and potassium lost by passing out in the slag be kept within commercial limits.

To obtain the best operating results, my invention contemplates the treatment of the combined phosphorus and potash bearing elements and carbon in an electric furnace in accordance with the principles laid down in my pending application Serial No. 388,822, which require the correct proportioning of the carbon content of the charge, the avoidance of open arcs, the maintenance of uniform furnace temperatures preferably between 1200° and 1500° C. by the constant diffusion of the electric heat through the slag bath, the preservation of a uniform depth of stock above the fusion zone, the automatic feed of the stock proportionate to the requirements of the fusion zone, and the preservation above the stock of a combustion space in which the evolved elemental phosphorus may be oxidized.

In addition to the foregoing I have found that special features are necessary for the contemporaneous volatilization and collection of both phosphorus and potash, whether or not in conjunction with the production of ferro-phosphorus. These are:

1st: The flux, which should be acid to treat phosphatic material and basic to treat potash materials, must be carefully calculated as to its proportions of lime and silica so that a minimum of phosphorus and potassium will be carried out of the furnace in the slag.

2nd: The phosphorus must be reduced then volatilized in the form of elemental phosphorus and subsequently oxidized to  $P_2O_5$  with which volatilized potassium combines to produce a compound of phosphoric acid and potash highly valuable for fertilizers and other uses.

I will now describe my invention with special attention to all limitations of the

various steps and features involved that are essential to its commercially and technically successful operation, and in such conciseness that those skilled in the art may actually be 5 enabled to successfully practice it.

In making up and proportioning my charge, I take a given quantity of any natural phosphate, consisting of the phosphorus bearing element, tricalcic phosphate, and 10 I take into account the accompanying silica, alumina, iron oxide, and magnesia. I then take potassium bearing shale or other potassium bearing rock, and add it to the charge in such quantity that the total silica of the 15 two above materials, of the molecular proportions corresponding to  $(CaO)_3 (SiO_2)_2$ , which corresponds to a quantitative ratio of 1.4 CaO to 1.0  $SiO_2$ . If magnesia be present in the mixture in quantity greater than 20 5 per cent of the weight of the total silica and lime added together, it is calculated into the flux charge in the same molecular ratio as that of the silica and lime or that of  $(MgO)_3 (SiO_2)_2$ , which corresponds to the 25 quantitative ratio of 1.0 part of MgO to 1.0 part of silica. The alumina present which usually is between 5 and 16 per cent of the total lime and silica together is in such case neglected in the flux calculation, be- 30 cause by actual practice I have found that the desired reactions and fluidity of the slag is little influenced by said alumina in said proportions.

The above described calculation of flux is 35 not based upon any assumptions or chemical theories of what the behavior of such proportioned slags will be under the conditions prevailing in conducting the herein- 40 described process but are the carefully noted results of actual practice in a commercial size unit of operation of said herein- 45 described process over a period of sufficient time to prove beyond doubt the effectiveness there- 50 of. I have determined by said actual prac- tice that, when smelting a charge in an elec- 55 tric furnace as in the herein- 60 described process, the above described composition of slag will be of the desired fluidity for the successful operation of the electric furnace under essential conditions for carrying out the herein- 65 described process, and that said slag will carry out of said furnace the minimum quantity of the phosphorus and potassium charged into and smelted in said furnace.

For the volatilization of phosphorus alone from natural phosphates and the practical elimination of phosphorus from the slag, there should be present in the charge in the 60 smelting furnace, an excess of silica, over and above that required to combine with all the lime present in the ratio of  $(CaO)_3 (SiO_2)_2$ , thus producing a so-called acid 65 slag. On the other hand, to set free and volatilize potassium compounds from their

associated rocks, there should be present an excess of lime over and above that required to combine with all the silica and alumina present in the total smelting charge, thus producing a so-called basic slag. Both theories 70 of slag characteristics are correct for each above specific case, taken separately, other conditions being properly provided. How- 75 ever, it is obvious that, when smelting the two above described materials for the pur- 80 pose of jointly freeing and volatilizing both potassium and phosphorus compounds, it is impossible to have a slag both acid and basic i. e., with both an excess of lime and an excess of silica. But, regardless of as- 85 sumptions or theories of the chemistry of the silicates and phosphates at high tempera- 90 tures, which in the present state of the sci- ence is not explicative of phenomena occur- 95 ring therein, I have discovered, practiced and proven that a lime, silica-alumina-mag- 100 nesia ratio of the above described compo- sition will, within the ratios and ranges specified fulfil the requirements for the suc- 105 cessful conductance of the herein- 110 described process.

To the charge of natural phosphate and shale or other natural potash bearing rocks, proportioned as above described I add car- 95 bon preferably in the form of finely divided coke, in quantity necessary to reduce all of the phosphorus and iron in charge. This carbon calculation is based upon the hypo- 100 thetical chemical equations:



I have found by actual commercial prac- 105 tice that, when less carbon is added than that required by the above equations, a con- siderable portion of the phosphorus and even iron passes into the slag unreduced. Also when any appreciable excess of car- 110 bon above that required and calculated by the above equations is used in the charge, said carbon excess accumulates in the fur- nace, and causes great irregularity in fur- 115 nace operation, destroying possibility of electrical control, thus causing overheating and contaminating fumes of  $SO_2$  and other constituents of the charge to be evolved, and defeating all other features of control of the 120 process herein- 125 described which make it a commercial operation.

With the above described furnace charge, I proceed with the operation by keeping the furnace charged continuously and uniformly over its entire surface of activity and maintaining the current flow entirely within the slag, and avoiding open arcs which cause a volatilization of the various constituents of the charge such as iron, lime, silica, mag- 125 nesia and alumina, which volatilized ma- 130

terials pass out of the furnace with the gases as fume and cause clogging of the gas mains and collecting equipment to such an extent as to require long interruptions of the operation and cleaning the entire gas system.

Furthermore, such volatilization of the above components of the stock disturb the balance in the proportion of the calculation of the reacting components, thus destroying 10 a principal factor of control which determines the success of the operation.

I have further found by actual and accurate measurements that the temperature of the slag within the operating furnace hereinbefore described must be maintained below 1450° C., and should preferably be between 1200° and 1350° C., and further that the temperature within the furnace must be gradually controlled so that each successive section of 20 the stock within furnace, from the slag to the top of the charge is of a lower temperature than that section above which it lies. When the temperature within the furnace rises above 1450° C., or when the temperature of 25 any portion of the charge within the furnace attains a temperature higher than that of the portion of the charge below it, the hereinbefore described phenomena of volatilized fume consisting of silica, alumina, lime and 30 magnesia occurs, and the electrical control of the furnace becomes so erratic as to be uncontrollable with any degree of uniformity. This is probably due to the great fluidity and boiling of slag from its superheating, 35 or from the increased conductivity of said slag resultant of such increased temperature, which produces arcing in the electric current flow, and intense heating of the charge by such superheating. In such state the slag 40 will present no definite plane of contact for the tips of the electrodes, thus producing violent surging of the flow of the current with arcing and breaking of the current, and creating irregular and heterogeneous 45 zones of excessive heating.

The accumulation of excessive carbon in the furnace from using an excess over that required for combining with the oxygen in combination with the phosphorus and iron 50 present in the charge and to form CO, will cause the formation of open arcs and overheating of the slag, producing the objectionable conditions above described. Hence the importance of maintaining the carbon ratio 55 as aforescribed. By the "oxygen in combination with the phosphorus and iron," I mean only the oxygen combined directly with the phosphorus or iron, as  $P_2O_5$ ,  $FeO$ ,  $Fe_2O_3$ ,  $Fe_3O_4$ , etc., and not that oxygen 60 which exists in combinations with other bases, such as  $CaO$ ,  $SiO_2$ , etc., with which the respective phosphorus and iron oxides may be in further chemical combination.

On the other hand, I have found, by the 65 maintaining of the regular and uniform

charging of said furnace and further maintaining the temperature of the slag within said furnace between 1200° and 1350° C., that a regular and continuous flow of current will be maintained, and that the phosphoric acid, as oxidized from the elemental phosphorus evolved or the potassium so evolved will also be passed out of the combustion chamber, in a state practically free from admixture of any accompanying fume 70 of silica, alumina, lime and magnesia, or other constituents of the stock other than those desired, and that the clogging of mains and of the other portions of gas, conducting or treating system will be eliminated, and that so long as the process is conducted with the temperature of the slag between 1200° and 1350° C., and the gradually lowering temperatures of the successive 75 layers of charge within the furnace from the slag upward is maintained the operation may proceed with uniformity, regularity, and continuity, and that the phosphoric acid oxidized from the elemental phosphorus evolved can be collected in a very pure 80 state and practically free from the contamination and interruption of operation by any accompanying fume and condensation product of silica, alumina, magnesia or constituents of the charge other than phosphorus or potassium compounds as desired. 85

I have further found and operated upon a commercial scale over a considerable period of modification of the principles of the aforescribed process in the production 100 of ferro-phosphorus, and have further found very distinct advantages to be gained thereby.

I take natural phosphate shale or other potassium bearing silicate rock, and carbon, in the proportions aforescribed, I then add iron in proportion to the phosphorus to produce the desired ferro-phosphorus. I have further found that in the production of ferro-phosphorus, by this means, a portion 105 of the phosphorus is always volatilized. The proportion of the total phosphorus volatilized is dependent upon the quantity and physical state of the iron present with the charge to absorb the phosphorus as reduced. For instance, if enough iron is present in the charge so that an alloy containing eighteen 110 per cent phosphorus is produced, there will be about ten per cent of the total phosphorus volatilized; and if enough iron is present in the charge so that an alloy containing twenty per cent phosphorus is produced, there will be about fifty per cent of the total phosphorus volatilized. The above figures will 115 vary somewhat depending upon the physical condition of the charge and certain inherent characteristics of the individual furnace construction and operation. But for any given lot of commercially available raw materials and any individual furnace, this 120

factor of phosphorus volatilization may be determined. Now by taking any given charge of natural phosphate, potash bearing silicate rock and carbon, I can by experiment determine, how much of the phosphorus contained in the charge will be absorbed by a given quantity of iron added to the charge and how much will be volatilized. I can then add enough iron to the given charge to absorb sufficient of the phosphorus so that a predetermined quantity of phosphorus will be volatilized, which predetermined quantity will be in such ratio to the potassium volatilized in the smelting charge, that, upon oxidation of the volatilized elemental phosphorus, and its combination, which occurs simultaneously with its collection, with the volatilized potash, there will be produced a definite chemical compound of potassium phosphate. In this way this process may be used for the production of a definite compound of potassium phosphate.

It is evident that in commercially available raw materials, the natural phosphates will contain varying proportions of phosphorus, silica, and lime, and the potassium bearing shales or other rock will contain varying proportions of potassium, silica, alumina and lime. Commercially available carbon reducing agent materials will also contain varying proportions of silica, alumina, lime and magnesia. Therefore with the number of variables effecting the above operation, it is self evident that a coincidence of proportions of contents of the governing constituents, so that, the ratio of the silica and lime will be in the ratios aforescribed, and also the ratio of the potassium and phosphorus in the proportions that exist in potassium phosphate, is not commercially possible. However with my process, iron, by proportioning the commercially available natural phosphate and potassium bearing silicate rock so as to produce the requisite character of slag, and by adding to this charge, including the reducing carbon, sufficient iron to absorb a portion of the phosphorus, which I will top out of the furnace as ferro-phosphorus, volatilize and oxidize the remaining phosphorus in predetermined proportion necessary to produce, with the potassium volatilized, a definite compound of potassium phosphate. At the same time in controlling the phosphorus volatilized by absorbing said predetermined portion with iron in the smelting charge, I will have produced a commercial product, and may make either the ferro-phosphorus or the potassium phosphate the principal product.

In case I produce ferro-phosphorus by the aforescribed process, I may consider in its commercial aspect that the potassium bearing shale is added in lieu of the silicious flux to the natural phosphate, in which case, with the properly proportioned charge as afore-

described, the potassium will be volatilized and collected along with the phosphorus oxides, which will considerably lower the cost of ferro-phosphorus production.

Furthermore in either case of the production of potassium phosphate or potash and phosphoric acid mixtures, or of ferro-phosphorus, and the collection of the potash and phosphoric acid, the collection of the phosphoric acid is greatly facilitated by the presence of the potash.

The phosphoric acid and potash may be separated from the accompanying gases by any of several methods such as electrical precipitation, absorption towers, or, since there will usually be an excess of phosphoric acid with the potash, ammonia gases may be passed into the potash and phosphoric acid bearing gases after withdrawing them from the furnace, thus combining the ammonia with the phosphoric acid and producing a complete fertilizer containing chemically combined ammonium potassium phosphate, in a dry powder direct and ready for distribution and use.

Having thus described my invention, what I claim as new and desire to secure by Letters Patent, is:—

1. The hereindescribed process, which consists in smelting in an electric furnace phosphate and potash bearing materials, with carbon in approximately the ratio required to combine with the oxygen combined in the charge with the phosphorus and iron present to form  $CO$ , oxidizing the evolved elemental phosphorus, causing the resultant phosphoric acid to combine with the evolved potash, and recovering the resultant compound of phosphorus and potash.

2. The process according to claim 1, in which the reduction is conducted at temperatures ranging from  $1200^{\circ} C.$  to  $1500^{\circ} C.$ , and in the absence of open arcs.

3. The process according to claim 2, in which the stock depth above the fusion zone is maintained substantially constant and of gradually decreasing temperature upwardly from the fusion zone.

4. The process according to claim 1, in which the phosphorus is evolved as elemental phosphorus and oxidized in the presence of the volatilized potash, which combines therewith to form a compound of potash and phosphorus.

5. The hereindescribed process for the recovery of compounds of phosphorus and potash, which consists in charging potash bearing shale with phosphatic material and a carbon reducing agent in ratio required for direct reduction of  $P_2O_5$  in said phosphatic materials in an electric furnace, smelting the mixture, oxidizing the volatilized phosphorus in the presence of the volatilized potash, and recovering the compound of potash and phosphorus.

6. The process according to claim 5, in which the total lime and silica in the charge shall be in the approximate molecular ratio of  $(\text{CaO})_3$  to  $(\text{SiO}_2)_2$ .
- 5 7. The process according to claim 5, in which the flux shall comprise silica and lime in the ratio of 1.4 parts of lime to 1.0 of silica.
8. The process according to claim 7, in 10 which magnesia in excess of 5 per cent is calculated into the flux charge in the same ratio as silica.
9. The herein-described process for the joint production of ferro-phosphorus and 15 compounds of phosphorus and potash, which consists in smelting in an electric furnace phosphatic material and iron with only sufficient carbon to reduce the iron and liberate the phosphorus, and with a silicious flux in 20 the form of a potash bearing silicate.
10. The process according to claim 9, in which potash bearing shale is used as the source of silicious flux and its quantity is proportioned to produce a flux containing 25 substantially 1.4 parts of silica to 1.0 parts of lime.
11. The herein-described process for producing potassium phosphate, which consists in charging a smelting furnace with phosphate and potash bearing materials and a reducing agent, and adding iron sufficient 30 to absorb the phosphorus content of the charge in excess of that required to com-
- bine with the potash content of the charge and form potassium phosphate. 35
12. The process according to claim 11, in which the iron and combined phosphorus are tapped from the furnace as ferro-phosphorus and in which the volatilized phosphorus and potash are combined as the 40 evolved phosphorus is oxidized, and recovered as potassium phosphate.
13. The herein-described process for the production ammonium potassium phosphate, which consists in smelting phosphate and 45 potash bearing materials in the presence of carbon in an electric furnace, oxidizing the evolved elemental phosphorus to form  $\text{P}_2\text{O}_5$ , combining the volatilized potash with the  $\text{P}_2\text{O}_5$ , combining ammonia with the free 50 phosphoric acid, and recovering ammonium potash phosphate.
14. The process according to claim 13, in which the constituents of the charge are proportioned to give an excess of  $\text{P}_2\text{O}_5$  gases 55 above that needed to form potassium phosphate, and this excess of phosphoric acid is used to fix the ammonia in ammonia gas added to the mixture of  $\text{P}_2\text{O}_5$  and potassium phosphate to form as a resultant product 60 ammonium potassium phosphate.

In testimony whereof I affix my signature.

BETHUNE G. KLUGH.

Witness:

NOMIE WELSH.